

[54] METHOD OF MAKING LIGHT GAGE  
MEMBERS OF UNALLOYED LOW CARBON  
STEEL SHEETS

[75] Inventor: Andor Mandoki, Budapest, Hungary

[73] Assignee: "Licencia" Talalmanyokat  
Ertekesito Vallalat, Budapest,  
Hungary

[22] Filed: Oct. 30, 1972

[21] Appl. No.: 301,814

## Related U.S. Application Data

[63] Continuation of Ser. No. 815,889, April 14, 1969,  
abandoned.

## [30] Foreign Application Priority Data

Apr. 19, 1968 Hungary ..... MA 1829

[52] U.S. Cl. ..... 148/12.4; 148/36; 148/143

[51] Int. Cl. ..... C21d 9/46

[58] Field of Search ..... 148/143, 144, 145, 146,  
148/147, 153, 36, 12.4, 2, 3

## [56] References Cited

## UNITED STATES PATENTS

3,410,734 11/1968 Taylor ..... 148/143

## OTHER PUBLICATIONS

Metals Handbook, Vol. 2, 8th Edition, 1964, pages  
36-46.

Primary Examiner—R. Dean

Attorney, Agent, or Firm—Young &amp; Thompson

[57]

## ABSTRACT

Thermal hardening is applied to the material of light gage cold-formed members made of unalloyed low carbon steel sheets having a carbon content not greater than 0.50 percent and a thickness not greater than 7 millimetres. Thermal hardening consists in quenching such steels from a temperature in the austenitizing range below the  $M_s$  temperature of starting martensite formation, holding the steel at such temperature until transformation is completed and then cooling it down to room temperature. By such method, an increase by 100 to 200 percent of the yield point may be obtained without distortion of the member. This seems to be due to the nose of the TTT-curve of beginning martensite formation being cut by the cooling curve so that softer crystal structures such as pearlite and bainite are formed which provide for absorbing residual stresses during martensite formation.

10 Claims, 8 Drawing Figures





Fig.1



Fig.3



Fig.4



Fig.5

SHEET 2 OF 2



Fig.2



Fig.6



Fig.7



Fig.8

## METHOD OF MAKING LIGHT GAGE MEMBERS OF UNALLOYED LOW CARBON STEEL SHEETS

This is a continuation of application Ser. No. 815,889, filed Apr. 14, 1969, and now abandoned.

### BACKGROUND OF THE INVENTION

This invention refers to methods of making light gage members of unalloyed low carbon steel sheets by employing thermal hardening.

Thermal hardening is generally substituted for conventional quenching and tempering in order to obtain improved mechanical properties such as high ductility or notch toughness at a given high hardness and/or to decrease the likelihood of cracking and distortion and thus to employ only two processing steps instead of conventional quenching and tempering which is a three step operation.

Various methods of thermal hardening of steel have been developed and are known in the art such as austempering, martempering or marquenching and patenting.

Austempering of steel means to heat it to a temperature within the austenitizing range from where it is quenched in a bath of constant temperature above the  $M_s$  point or temperature of rapid conversion of austenite in martensite. The steel is maintained in the bath at such temperature until the austenite is isothermally transformed to bainite whereafter it is left to cool down to room temperature, usually in still air. Austempering is described in detail in the specification of U.S. Pat. No. 1,924,099 to Edgar C. Bain et al. which is hereby incorporated by reference. Austempering has modified forms as well in which bainite is mixed with pearlite. Another form of modified austempering is patenting which is the heat treating of wires or rods providing a combination of moderately high strength and high ductility.

As to martempering, it consists in quenching a steel from the austenitizing range to a temperature in or slightly above the martensite range and holding the steel at such temperature until its whole cross-sectional area is uniformly heated whereafter the steel is permitted to cool at a moderate rate. Hereby, fairly uniform martensite formation is obtained throughout the work piece and yet excessive amounts of residual stresses are avoided. Martempering has likewise its modified forms which are distinguished from standard martempering only by a lower temperature of the quenching bath. Such modified martempering permits to employ faster cooling rates which is important for steels of lower hardenability.

All these methods of thermal hardening are described in detail in "Metals handbook" of the American Society for Metals, Metals Park, Ohio, 8th edition, 1964, vol. 2, hereby incorporated by reference which has widely been taken recourse to when composing the present text.

As is known, with austempering a work piece is quenched past the nose of the TTT-curve (time-temperature transformation curve). If the cooling curve intersects the nose of the TTT-curve true austempering is already impossible. Such intersection is unavoidable if the carbon content of the steel is too low and its surface-to-mass relation too little since then extremely fast pearlite reaction times have to be reckoned with and the cooling curves cannot avoid the nose of the TTT-curve of starting conversion either practi-

cally (too small time allowance for quenching) or theoretically (no such allowance at all). Due to such limitations, the domain of plain carbon steels adaptable to austempering is restricted to carbon contents not less than 0.50 % carbon up to 1.00 % and a minimum of 0.60 % manganese. By increasing the austenitizing temperature the nose of the TTT-curve could be caused to shift to the right whereby compositions or section sizes that would otherwise be border line for austempering would be enabled to be processed. However, coarser grain sizes resulting from increased austenitizing temperatures might entail deterioration of otherwise desired mechanical properties such as ductility and yield point. For similar reasons, carbon steels of lower carbon content will be restricted to proportionately lesser thicknesses and 5 millimetres are about the upper limit.

With modified practice of austempering, the process differs from true austempering in that the quenching rate is not rapid enough to avoid the nose of the TTT-curve which is intersected by the cooling curve substantially above the  $M_s$  temperature so that fine pearlite will be formed.

Likewise, steels chosen for martempering must contain sufficient amount of carbon to move the nose of the TTT-curve to the right so as to allow sufficient time for quenching a work piece past it. Actually, steels selected for martempering must have a carbon content somewhat higher than for conventional (uninterrupted) quenching which means again that plain carbon steels of lower carbon content are unsuitable for both standard and modified martempering since with such steels the nose of the TTT-curve would be intersected and the formation of martensite would be frustrated. For similar reasons, the thickness of the work piece must not exceed an upper limit (generally 5 millimetres) either.

Thus, according to the prior art, thin steel members of low carbon content which cannot be hardened by the conventional method of austenitizing, quenching and tempering because of their low carbon content and the danger of distortions caused by residual stresses, cannot be thermally hardened by standard or modified austempering either the use of which is restricted to plain carbon steels having a carbon content more than 0.50 percent. Moreover, they cannot be thermally hardened by martempering, standard or modified, either because of their low hardenability.

On the other hand, it is known that unalloyed low carbon steels are considerably less expensive than similar steels of higher carbon content. Therefore, it would be desirable to process such steels into light gage cold-formed members and particularly in sections since there is great demand for disconnectable metal structures composed of such members and erectable in situ. Obviously, considerable savings as to costs, weight and space might be obtained if such metal structures could be made of light gage cold-formed members of low carbon content. Hitherto, however, unalloyed low carbon steels have been excluded from the use for such purpose because of their relatively low yield point and more particularly due to the poor relation between yield point and associated tensile strength which are the basis of dimensioning such structures.

### SUMMARY OF THE INVENTION

The main object of the present invention is to provide a method by which the yield point of such members can

considerably be improved so as to permit their use in constructions which hitherto have required steels of higher carbon contents. The invention is based on the discovery that contrary to the view mirrored in the prior art, even such steels can be thermally hardened without detrimental consequences if, on the one hand, the nose of the TTT-curve of beginning transformation is not only intersected but deliberately crossed by the cooling curve and, on the other hand, quenching is pushed beyond the  $M_s$  temperature yet not far enough to reach the temperature range of conventional quenching responsible for the formation of brittle martensite. Sufficient time is then allowed for the conversion of austenite still present to be converted in martensite forming at such temperature whereafter the member is permitted to cool down to room temperature.

At present, it is believed that the favourable results as to increased yield point and absence of distortions obtained by such method are due to the formation of substantial amounts of less brittle martensite beneath the  $M_s$  point and to the formation of softer crystal structures such as pearlite and bainite during the crossing of the TTT-curve nose prior to the formation of martensite, softer crystal structures and martensite being in favourable mutual proportions probably due to the cooling curve being steeper because of lower quenching temperature (as if the first section of the cooling curve had been rotated in the clockwise direction). Thus, the method according to the invention is intermediate between austempering and modified martempering in that final temperature of quenching lies beneath the  $M_s$  point as distinguished from austempering, and in the course of quenching softer crystal structures are formed because of crossing the nose of the TTT-curve of beginning transformation as distinguished from modified martempering (see e.g. FIG. 1 "Austempering" on page 57 and FIG. 1 "Modified martempering" on page 37, respectively, of "Metals Handbook"). Experiments have proved that such crossing of the nose of the TTT-curve of beginning transformation is ensured if members subjected to the suggested thermal hardening are made of unalloyed carbon steel sheets the carbon content of which is not greater than the aforesaid critical value of 0.50 percent and the sheet thickness is not greater than 7 millimetres which means that even the thickness range could be extended beyond the hitherto known upper limit of about 5 millimetres.

Summarily, the invention is concerned with a method of making light gage cold-formed members and more particularly sections of unalloyed low carbon steel sheets having a carbon content not greater than 0.50 percent and a thickness not greater than 7 millimetres wherein the improvement consists in the step of thermally hardening the members by means of quenching the same from a temperature above the critical temperature range to an intermediate temperature below that at which rapid conversion of austenite to martensite is obtained but above that at which conversion is not rapid enough to cause the austenite to be converted in brittle martensite, and thereafter maintaining the quenched steel at this intermediate temperature for a time interval sufficient to obtain conversion of the remaining austenite to pure martensite characteristic for the temperature of heat treatment, and then cooling to atmospheric temperatures. The term "cold-formed

member" in the present specification and in the appended claims is meant to cover individual constructional parts as well as small, thin sections made by bending sheet or strip steel in roll-forming machines, 5 press brakes or bending brakes. Furthermore, the term "sheet" is meant to cover plates and strips as well, the difference being, principally, a matter of thickness and width of material whether or not the material is furnished in flat form or in coils.

#### BRIEF DESCRIPTION OF THE DRAWING

The invention will be described hereinafter in closer details, by taking reference to the accompanying drawings in which:

FIG. 1 shows a time-temperature transformation diagram symbolic of the thermal hardening employed with methods according to the invention.

FIG. 2 is a similar diagram showing actual TTT-curves of various steels having carbon contents within the range prescribed by the invention.

FIG. 3 shows a member made by a method according to the invention.

FIGS. 4 to 8 show sections of various shapes.

Same reference characters refer to similar details 25 throughout the drawings.

In the drawings, FIG. 1 illustrates the basic principle of the method according to the invention. Lines I and II represent broadly the envelopes of TTT-curves of starting and complete transformations, respectively, 30 critical temperature  $Ae3$  represents the range of critical temperatures of steels having carbon contents within the scope of the present invention. Line  $M_s$  is a respective symbol of temperatures below which martensite formation is due. Q refers to the cooling curve 35 characteristic of quenching such steels from above critical temperature  $Ae3$  below  $M_s$  temperature, then maintaining it at constant temperature and, finally, cooling it to room temperature. It is seen that the envelope I of TTT-curves of beginning transformation is already cut at its nose. Consequently, it is practically impossible to quench such steels rapidly enough to pass the nose of their TTT-curves of beginning transformation. Thus, formation of other crystal structures than martensite will take place prior to martensite formation. 40 On the other hand, an intersection with the envelope II of TTT-curves of complete transformation has to be avoided, otherwise only little martensite formation would occur. Experiments have shown that such requirement will be met with if sheet thicknesses 45 greater than 7 millimetres are dismissed. Thus, with steel members having a carbon content not greater than 0.50 percent and a thickness not greater than 7 millimetres, the cooling curve Q will always cross the nose of the respective TTT-curve of beginning transformation without intersection with the associated TTT-curve of complete transformation as illustrated for the envelope I both branches of which are intersected by the cooling curve Q, the latter being steep enough not to intersect envelope II.

The significance of such double intersection or crossing is that at the first intersection A the austenite will begin to convert in softer crystal structures in correspondence with decreasing temperature until the second intersection B is reached. In this period, pearlite and bainite will be formed. After the second intersection B the remaining austenite will stay unchanged until the  $M_s$  temperature is passed (point C) whereupon

conversion of the remaining austenite into martensite will set in. Since such conversion takes place at a constant temperature — broadly between 150° and 470° centigrade — elevated with respect to the temperature where brittle martensite is formed (as with conventional quenching), the remaining austenite becomes converted into relatively soft martensite, conversion being completed at the intersection of the horizontal section of the cooling curve Q with the envelope II of TTT-curves of complete transformation (point D). Thereafter, cooling to room temperature may be carried out along the final section of the cooling curve Q, a substantial allowance of time to start, such cooling being provided for with regard to the uncertainty of the course of the TTT-curves of complete transformation at such medium temperatures. Thus, the crystal structure of the member will consist, besides of softer elements such as pearlite and bainite formed between points A and B, of a substantial portion of soft martensite. The former are believed to account for the absence of distortions during the formation of the latter whereas the presence of substantial amounts of soft martensite seems to be responsible for an unsuspected increase of the yield point. Obviously, the presence of bainite contributes to the increase of the yield point and, vice versa, the formation of soft rather than brittle martensite may result in avoiding residual stresses. Thus, increased yield point will be obtained without significant distortions which is the main object of the present invention.

FIG. 2 shows the actual TTT-curves of beginning and complete transformations for steels having carbon contents of 0.50 % (dash-and-dot lines), 0.35 % (dotted lines) and 0.15 % (dashed lines), respectively, and, thus, covering the whole range of pertinent steel compositions. It is seen that the noses of all TTT-curves of beginning transformation are crossed by the cooling curve Q, and none of the TTT-curves of complete transformation is intersected by the same which are the theoretical conditions for the working of the method in accordance with the invention.

#### DESCRIPTION OF THE PREFERRED EMBODIMENTS

Various examples of steels selected and heat treated or thermally hardened in compliance with the present invention are set forth in the following four tables which group altogether nineteen embodiments stating decisive data of heat treatment and characteristic data of mechanical properties. All steels are plain carbon steels with the usual amounts of silicon, sulphur and phosphorus. They differ from one another as to their contents of carbon and manganese, which rule the subdivision into groups. The lowest carbon content is 0.15 percent for steels of group I. The two next groups include steels of carbon contents of 0.25 and 0.35 percent, respectively. Finally, group IV lists steels having a carbon content of 0.45 percent which is almost the maximum amount of carbon permissible with steels selected for the purpose of the invention. The content of manganese correspondingly decreases as the carbon content approaches its upper limit though, obviously, other manganese contents might be chosen within the limits of such constituent in plain carbon steels as will be apparent to the skilled art worker.

#### GROUP I OF EXAMPLES

Carbon: 0.15 %  
Manganese: 0.80 %

| Example                                 | 1   | 2   | 3   |
|-----------------------------------------|-----|-----|-----|
| Thickness in mm                         | 0.5 | 1.5 | 2.5 |
| Austenitizing temperature in °C         | 950 | 950 | 950 |
| Ms temperature in °C                    | 460 | 460 | 460 |
| Temperature of quenching in °C          | 400 | 350 | 350 |
| Theoretical quenching time in sec       | 30  | 55  | 50  |
| Actual quenching time in sec            | 200 | 300 | 300 |
| Initial tensile strength in kg/mm²      | 37  | 37  | 37  |
| Final tensile strength in kg/mm²        | 80  | 70  | 60  |
| Initial ductility in %                  | 30  | 30  | 30  |
| Final ductility in %                    | 18  | 20  | 22  |
| Initial yield point in kg/mm²           | 22  | 22  | 22  |
| Final yield point in kg/mm²             | 60  | 50  | 40  |
| Percentual increase of yield point in % | 173 | 127 | 82  |

#### GROUP II OF EXAMPLES

Carbon: 0.25 %  
Manganese: 0.65 %

| Example                                 | 4   | 5   | 6   | 7   | 8   | 9   |
|-----------------------------------------|-----|-----|-----|-----|-----|-----|
| Thickness in mm                         | 2.0 | 2.0 | 2.0 | 2.0 | 2.0 | 2.0 |
| Austenitizing temperature in °C         | 910 | 910 | 910 | 910 | 910 | 910 |
| Ms temperature in °C                    | 420 | 420 | 420 | 420 | 420 | 420 |
| Temperature of quenching in °C          | 170 | 200 | 250 | 300 | 350 | 400 |
| Theoretical quenching time in sec       | 300 | 250 | 180 | 110 | 65  | 35  |
| Actual quenching time in sec            | 600 | 600 | 500 | 400 | 300 | 300 |
| Initial tensile strength in kg/mm²      | 45  | 45  | 45  | 45  | 45  | 45  |
| Final tensile strength in kg/mm²        | 125 | 115 | 105 | 90  | 80  | 70  |
| Initial ductility in %                  | 20  | 20  | 20  | 20  | 20  | 20  |
| Final ductility in %                    | 5   | 6   | 7   | 8   | 14  | 16  |
| Initial yield point in kg/mm²           | 25  | 25  | 25  | 25  | 25  | 25  |
| Final yield point in kg/mm²             | 90  | 85  | 80  | 70  | 60  | 55  |
| Percentual increase of yield point in % | 260 | 240 | 220 | 180 | 140 | 120 |

#### GROUP III OF EXAMPLES

Carbon: 0.35 %  
Manganese: 0.65 %

| Example                            | 10  | 11  | 12  | 13  | 14  | 15  |
|------------------------------------|-----|-----|-----|-----|-----|-----|
| Thickness in mm                    | 2.0 | 2.0 | 3.0 | 3.0 | 3.0 | 6.0 |
| Austenitizing temperature in °C    | 870 | 870 | 870 | 870 | 870 | 870 |
| Ms temperature in °C               | 385 | 385 | 385 | 385 | 385 | 385 |
| Temperature of quenching in °C     | 300 | 350 | 250 | 300 | 400 | 250 |
| Theoretical quenching time in sec  | 120 | 75  | 180 | 120 | 40  | 180 |
| Actual quenching time in sec       | 400 | 300 | 500 | 400 | 300 | 500 |
| Initial tensile strength in kg/mm² | 55  | 55  | 55  | 55  | 55  | 55  |
| Final tensile strength in kg/mm²   | 115 | 105 | 105 | 90  | 80  | 80  |
| Initial ductility in %             | 17  | 17  | 17  | 17  | 17  | 17  |
| Final ductility in %               | 8   | 9   | 10  | 12  | 14  | 16  |
| Initial yield point in kg/mm²      | 30  | 30  | 30  | 30  | 30  | 30  |

-Continued

## GROUP III OF EXAMPLES

Carbon: 0.35 %  
Manganese: 0.65 %

| Example                                    | 10  | 11  | 12  | 13  | 14  | 15  |
|--------------------------------------------|-----|-----|-----|-----|-----|-----|
| Final yield point<br>in kg/mm <sup>2</sup> | 85  | 80  | 80  | 70  | 60  | 60  |
| Percentual increase<br>of yield point in % | 184 | 167 | 167 | 134 | 100 | 100 |

## GROUP IV OF EXAMPLES

Carbon: 0.45 %  
Manganese: 0.50 % (maximum)

| Example                                           | 16  | 17  | 18  | 19  |
|---------------------------------------------------|-----|-----|-----|-----|
| Thickness in mm                                   | 2.0 | 2.0 | 4.0 | 7.0 |
| Austenitizing temperature<br>in °C                | 850 | 850 | 850 | 850 |
| Ms temperature in °C                              | 350 | 350 | 350 | 350 |
| Temperature of quenching<br>in °C                 | 330 | 330 | 330 | 250 |
| Theoretical quenching time<br>in sec              | 130 | 130 | 130 | 180 |
| Actual quenching time<br>in sec                   | 400 | 250 | 400 | 500 |
| Initial tensile strength<br>in kg/mm <sup>2</sup> | 65  | 65  | 65  | 65  |
| Final tensile strength<br>in kg/mm <sup>2</sup>   | 115 | 125 | 105 | 90  |
| Initial ductility in %                            | 14  | 14  | 14  | 14  |
| Final ductility in %                              | 9   | 8   | 12  | 14  |
| Initial yield point<br>in kg/mm <sup>2</sup>      | 35  | 35  | 35  | 35  |
| Final yield point<br>in kg/mm <sup>2</sup>        | 90  | 95  | 80  | 70  |
| Percentual increase<br>of yield point in %        | 157 | 199 | 129 | 200 |

In each of the nineteen cases, conventional salt baths have been used for quenching. Such baths are described e.g. in the above mentioned Metals Handbook.

Furthermore, in each case final cooling has been carried out in still air though water might be used as well. Then, a further increase of the yield point by 2 to 3 kilograms per square millimetres can be obtained due to the traces of remaining austenite being converted in brittle martensite.

The tables show that each embodiment is characterised by a considerable increase of the yield point with respect to values prior to heat treatment. Though such increase is obtained through the whole range of pertinent steel compositions, greatest values are associated with thicknesses between 1.5 to 4 millimetres (see group II, examples 4, 5 and 6 and group IV, examples 16 and 17) and/or with a carbon content not less than 0.15 percent (see group II, examples 4, 5 and 6).

Furthermore, the tables show that manganese contents not less than 0.5 percent have proved very favourable as to the percentual increase of the yield point as witnessed by all groups of examples.

The temperature of heating will preferably amount to 30° to 90° centigrade higher than the lowermost temperature limit of the austenitizing range. Though, as has been referred to, temperatures higher than that increase the quenching speed and thereby the strength, their grain coarsening effect outbalances the gain obtained by higher quenching speed. One of the favourable features of the invention is that usual austenitizing temperatures may be employed for obtaining the desired results.

FIGS. 3 to 8 show various members made by the method according to the invention. Basically, two

groups of such members may be distinguished. One group comprises individual parts such as the roller chain link plate shown in FIG. 3. The other group includes various sections, such as flat sections (FIG. 4), equal leg angles (FIG. 5), open or closed channel sections (FIGS. 6 and 7, respectively) or sections of special cross-sectional shapes such as shown in FIG. 8.

Flat sections as illustrated in FIG. 4 may be heat treated according to the present invention in continuous operation. Then, the material is furnished in coils and is passed through various treating stations in band form. The heat treated band may be wound up for storage or cold-formed and cut to predetermined lengths. In both cases heating, quenching and cooling is applied to the work material prior to shaping the cross-sectional area thereof.

On the other hand, individual parts such as the roller chain link plate shown in FIG. 3 or the sections shown in FIGS. 5 and 8 will preferably be heat treated groupwise. In such cases, the work material will be shaped or cold-formed and subdivided into predetermined lengths by means of cutting (see FIG. 6), prior to heating, quenching and cooling.

With both methods, the equipment necessary for continuous or groupwise heat treatment may be composed of units well known in the art for similar purposes and in a manner familiar with the skilled art worker. In this respect, reference is again taken to the above mentioned Metals Handbook.

I claim:

1. In a method of making light gage members of unalloyed low carbon steel sheets having a carbon content not greater than 0.50%, the steps of

heating a said member above the critical temperature thereby to form austenite, thermally hardening the member by quenching the same from a temperature above the critical temperature to an intermediate temperature of substantially 150° to 470° centigrade along a cooling line that crosses the nose of the time-temperature transformation curve, to convert only a portion of said austenite to pearlite and bainite, and thereafter maintaining the quenched steel at this intermediate temperature for a time interval sufficient to obtain conversion of the remaining austenite to pure martensite characteristic of the temperature of heat treatment, and then cooling to room temperature.

2. In a method of making members as claimed in claim 1 including the step of cold-forming the cross-sectional area of work material the further improvement of applying the heating, quenching and cooling to the work material prior to cold-forming of the cross-sectional area thereof in a continuous operation.

3. In a method of making members as claimed in claim 1 including the step of cold-forming the cross-sectional area of work material the further improvement of applying the heating, quenching and cooling to the work material groupwise after cold-forming its cross-sectional area.

4. In a method of making members as claimed in claim 1 the further improvement of employing steel sheets of a thickness of 1.5 to 4 millimetres for work material.

5. In a method of making members as claimed in claim 1 the further improvement of employing steel

sheets having a carbon content not less than 0.15 percent for work material.

6. In a method of making members as claimed in claim 1 the further improvement of employing steels for work material the manganese content of which is 0.5 to 1.0% by weight.

7. In a method of making members as claimed in claim 1 the further improvement of carrying out quenching from a temperature by 30° to 90° centigrade higher than the lowermost temperature limit of the austenitizing range.

8. In a method of making members as claimed in claim 1 the further improvement of effecting the final cooling in water.

9. In a method of making members as claimed in claim 1, the further improvement of performing said quenching in a salt bath.

10. In a method of making members as claimed in claim 1, the further improvement of maintaining the thickness of the members not greater than 7 millimeters.

\* \* \* \* \*

15

20

25

30

35

40

45

50

55

60

65